

United States Patent [19]  
Wessel

[11] 3,805,574  
[45] Apr. 23, 1974

[54] EQUIPMENT FOR EXTRUSION

[76] Inventor: Otto Wessel, Duisburg-Ungelsheim,  
Germany

[22] Filed: Jan. 21, 1972

[21] Appl. No.: 215,886

Related U.S. Application Data

[63] Continuation of Ser. No. 818,023, April 21, 1969,  
abandoned.

[52] U.S. Cl. .... 72/253, 72/265, 72/271

[51] Int. Cl. .... B21c 23/00

[58] Field of Search .... 72/253, 256, 265, 271;  
264/323; 425/812

[56] References Cited

UNITED STATES PATENTS

3,189,988 6/1965 Crane ..... 29/420.5

|           |         |                        |         |
|-----------|---------|------------------------|---------|
| 2,063,563 | 12/1936 | Sparks .....           | 72/265  |
| 1,664,990 | 4/1928  | Oehmig et al. ....     | 72/255  |
| 2,688,400 | 9/1954  | Ansel .....            | 72/254  |
| 3,109,202 | 11/1963 | Beckadolph et al. .... | 425/812 |
| 3,151,968 | 10/1964 | Wallar .....           | 425/812 |

Primary Examiner—Charles W. Lanham

Assistant Examiner—James R. Duzan

Attorney, Agent, or Firm—Smyth, Boston & Pavitt

[57]

ABSTRACT

A method for extrusion molding and equipment for carrying out the method is disclosed in which, prior to extrusion, porous blocks are compressed such that the density gradually increases from the interior to the exterior to force enclosed gas to flow in outward directions.

11 Claims, 3 Drawing Figures



PATENTED APR 23 1974

3,805,574

SHEET 1 OF 2

Fig. 1



Inventor:  
Otto Wessel

By Smith, Estes & Harrold,  
ATTORNEYS

PATENTED APR 23 1974

3,805,574

SHEET 2 OF 2

Fig.3



Fig.2



Inventor:  
Otto Wessel

By Smyth, Costow & Paris,  
ATTORNEYS

## EQUIPMENT FOR EXTRUSION

This is a continuation, of application Ser. No. 818,023, filed Apr. 21, 1969.

The present invention relates to method and apparatus for extrusion such as extrusion molding of work pieces having hollow or solid sections at rather high density, while using porous blocks as raw material and which, in turn, have been manufactured from powdery material. The invention, furthermore, relates to equipment coacting with such a block on basis of particular contour relationship including novel aspects for the blocks themselves.

In the recent past, it has become known to use metallic powder for extrusion molding. In particular, the powder is preformed or pressed into blocks and the blocks are extruded. The resulting reaction pressure arising during extrusion was found to be particularly favorable, and the degree of possible deformation is particularly high when such porous blocks are used as raw material. The extrusion is conducted at cold temperatures. However, the temperature should preferably be above the recrystallization temperature of the material.

It was found, however, that certain difficulties arise if one attempts to extrude directly from porous blocks for producing a rather compact final product. These difficulties arise particularly from the gases encapsulated in the pores or lodged between the grains of the powder. As a ram or plunger exerts pressure upon the powder, or the porous blocks which have been placed in the receiver portion of the extrusion apparatus, there is at first an increase in density, i.e., the compression reduces the porosity. Subsequent thereto, the compressed material begins to flow for extrusion through the extrusion nozzle of the die.

Gas still remaining in pores and cavities is very strongly compressed, and pressure therein may rise up to 5,000 or even as high as 15,000 atmospheres, depending upon the material that is being worked. This, of course, is true only if the gas could not escape. In case of large, porous blocks having relatively low relative density, considerable quantities of gas have to be removed, but usually only comparatively short periods of time are available for the gas removal. Moreover, the gas is to be removed under highly unfavorable flow conditions because the cells and pores establishing the porosity have rather small dimensions, establishing long and narrow flow paths. Moreover, extrusion molding equipment as commonly used has rather close tolerances so that further escape of gas is impeded, even inhibited.

The gas encapsulated in the pores has usually been used for heating. This gas as enclosed in the pores and compressed is heated during the compression, particularly after hot extrusion or during a subsequent heating process. This, in turn, may cause the extruded material to tear and to form enclosed bubbles in the final product.

It is now known to avoid the inclusion of gas during extrusion molding in that the porous blocks are clad in a sheet metal lining. The lining is closed through welding, and the resulting enclosure is finally hermetically sealed. Thus, the porous blocks are degassed prior to extrusion. The metallic lining is likewise extruded and protects the block against gas and lubricants from the outside. However, such a method is necessarily rather

expensive and is particularly not economical for easily reducible materials such as copper, nickel or iron.

Another way to avoid gas enclosure is known and is disclosed in British Pat. No. 1,008,250. According to this known method the blocks are formed with a rather low total volume of the pores. In accordance with the teaching of that British patent, the porous blocks are made from powder, preferably having grains of the size of 0.01 through 0.012 millimeters. The resulting blocks have a rather uniform, relative density of 80 to 90 percent. The principal difficulty with this method arises from the fact that treatment of such porous blocks with a gas down to the core, for example, a reduction of oxides in a gaseous atmosphere is practically not possible 15 economically as for such high densities the gas treatment requires too much time.

It is an object of the present invention, to provide a method and equipment for extrusion molding without incurring gas enclosures in the final product while using 20 porous blocks without outer lining or cover from which to extrude. In accordance with the invention, it is suggested to use uncovered blocks of open porosity and having a relative density of 50 to 80 percent and to compress such a block prior to extrusion flow of the 25 material such that the density increases progressively from the interior toward the outside. In particular, the block is compressed by applying force in a particular direction along a central axis of such a porous block, and the density is made to increase in radial outward 30 progression from the axis along which the force applying plunger moves.

The block and/or the plunger are appropriately shaped to obtain compression at gradual progression from the interior towards the outside to force the gas 35 out of compressed pores and into pores not yet or less compressed. Hence, the gas is forced to flow in radial outward direction, corresponding to the progression of the compression. In general, the invention resides in the providing of a controlled rate and spatial distribution 40 of compression such that the enclosed gas is forced to flow in the desired direction to be finally forced out of block and tool.

As compression is continued, the material extrudes 45 without carrying gas bubbles. The inventive method regarding the essentially radially progressing compression of the block can be practiced, for example, by perforating a solid block or by enlarging or widening a hollow block in the extrusion molding equipment. The 50 final product will then have hollow section.

The invention includes equipment for manufacturing dense and solid or hollow section pieces by means of extrusion molding from porous, uncovered blocks made of powdery material. Plunger and die member of the extrusion press have surfaces which face each other across the receiver cavity holding the block. These surfaces are relative inclined to each other with reference to an axis. As preferred construction, the plunger head is provided with a convex contour established, for example, by a conical or frustoconical protrusion. The die member is provided with a concave contour established, for example, by a conical or frustoconical indentation. Generally, the concave indentation is to be shallower (even completely flat) than the convexity by which the plunger head protrudes.

The extrusion press equipment is characterized in particular in that die member and plunger have frustoconically-shaped surfaces facing each other across

the receiver, whereby the base angles differ by approximately 10 to 30 percent; the base angle of the plunger head surface being the larger one. Preferably, the base angle of the frustoconical protrusion of the plunger is larger by 17° to 22° than the base angle of the coacting die member. The base angle of the frustoconical indentation of the die member itself may have an angle in the range of 0° to 15°, preferably 10°.

The difference in relative inclination of the coacting surfaces of plunger and die member causes force to be applied upon the porous blocks at first in a core zone along the axis of relative motion of plunger and die member. Hence, that central axial region of the porous block is compressed first. As compression pressure continues, the compression propagates from this central region in an outward direction. Gas contained in the pores is forced to escape corresponding to the progressing compression from the inner region toward the outer regions of the block.

The gas will collect near the outer, circumferential surfaces of the block, and in accordance with an additional feature of the invention the guiding surface for the plunger which slides along the receiver and closes the receiver cavity, is provided with shallow grooves. The collected gas can escape through these grooves and along the adjacent walls of the receiver. As pressure is increased upon the block, the gas is forced into these grooves. In accordance with another feature of the present invention, the outer surface of the die member engaging the receiving section of the extrusion molding equipment may likewise be provided with shallow grooves for removal of gas in an analogous manner.

For extrusion of a work piece having hollow profile, the plunger arrangement is provided with a mandrel as known, *per se*. The purpose thereof is to perforate the block inside of the extrusion equipment. In accordance with this feature of the invention, the mandrel is provided with a conical peak having an apex angle of 45° to 75°. It was found that best results can be obtained if the angle is about 60°.

The principle underlying the invention requires a compression gradient from the interior to the exterior of the compressed block prior to extrusion. This pressure gradient is obtainable through the particular angular relation between the two surfaces of plunger head and die member facing each other across the receiver cavity. However, it has to be observed that these two coacting surfaces engage different surface portions of the block. Therefore, the desired compression gradient can also be produced by an appropriate relationship between the block surfaces on one hand, and the two coacting surfaces of plunger head and die member.

It is, therefore, within the scope of the invention to produce the desired pressure distribution during compression in such a manner that the porous block is provided with at least one outwardly bulging front face. The bulging surface may preferably have the contour of a calotte. However, it is still preferred to provide the front face of the block with a frustoconical configuration. The base angle of this frustoconical protrusion of the block is preferably 10 to 30°. It was found to be particularly advantageous to preshape the block as a cylinder (possibly with at least one frustoconical or calotte-shaped axial end face), and to choose the geometrical dimensions thereof such that the ratio of cylinder height to diameter is at least 2.5:1.

It should be mentioned that British Pat. No. 1,008,250, referred to previously, basically discloses a plunger with a bulging head as well as a die with a particular inclination of its coacting surface. However, in this patent the several surfaces are inclined relative to each other such that a compression distribution results in which higher densities progress from outer to inner regions, therefore causing the gases to be firmly enclosed in the interior with little chance to escape.

10 While the specification concludes with claims particularly pointing out and distinctly claiming the subject matter which is regarded as the invention, it is believed that the invention, the objects and features of the invention and further objects, features, and advantages 15 thereof will be better understood from the following description taken in connection with the accompanying drawings in which:

FIG. 1 is an elevation and cross section view of a device for making hollow section work pieces in accordance with the preferred embodiment of the present invention;

20 FIG. 2 illustrates an elevation and section view of a device for making solid section work pieces in accordance with the method of the present invention; and

25 FIG. 3 illustrates a block as it is to be used preferably for practicing the method in accordance with the present invention.

The device and equipment illustrated in FIG. 1 comprises a base plate 13 having a bore 23 receiving the extruded material. Plate 13 supports the receiver 9, as well as the member 5, provided with the extrusion nozzle 51. Receiver 9, die member 5 and a plunger head 2, when inserted in the receiver, define the receiver cavity. The receiver contains a block 6. Block 6 is presumed to have been prepressed from powdery material and constitutes a porous block having relative density of 50 to 80 percent, preferably 65 to 75 percent.

30 A plunger 3 is provided above the block 6. The plunger 3 carries the head 2 having a frustoconically-shaped protrusion 1 to define a press surface of like designation. Thus, a frustoconically-shaped press surface faces the block 6, and through the receiver cavity the die member 5. A guiding surface 10 of plunger head 2 is provided with flat grooves 11 for permitting escape of the gas which has been squeezed out of the block 6. The gas escapes from the receiver cavity through grooves 11 along adjacent, upper portion of the wall of receiver 9. The die member 5 is likewise provided with flat grooves 12 facing the lower wall portion of receiver 9 to permit the escape of gas.

35 The surface 4 of die member 5 defining the contour of the bottom of the receiver cavity is funnel or conically-shaped, *i.e.*, the die member has a concavity defined by surface portions which are inclined toward center and extrusion nozzle 51, to likewise constitute a frustoconical surface.

40 The frustoconical protrusion surface 1 has a base angle  $\alpha$ , measured relative to an axial plane, the axis of the core being the common axis of the system defining also the direction of plunger movement and running through the center of the extrusion nozzle and of the core defined by surface 4. The frustoconical surface 4 has a base angle  $\beta$  relative to another axial plane. In accordance with the principle of the invention, the base angle  $\alpha$  is larger than the base angle  $\beta$  the difference being in the range between 10° and 30°. It is preferred to have a difference of 17°-22°. The base angle  $\beta$  itself

is preferably between  $0^\circ$  and  $15^\circ$ , an angle of about  $10^\circ$  being preferred. Hence, in preferred configuration angle  $\alpha$  has value between  $27^\circ$  and  $32^\circ$ .

The plunger 3 is provided in its interior with a mandrel 7 which is concentric to frustoconical surfaces 1 and 4. Mandrel 7 is provided with a conical peak 8 in order to provide block 6 with a central bore or if the block does already have a central bore to widen the bore, the apex angle of that peak,  $\gamma$ , is approximately  $60^\circ$ . FIG. 1 illustrates mandrel 7 in a position of initial insertion into block 6. The dashed lines 7', 8', respectively, show mandrel and peak in protracted position after perforation or widening.

In FIG. 2 similar parts are designated by like reference numerals. The embodiment of FIG. 2 differs from the embodiment illustrated in FIG. 1 in that the former is designed to extrude a string or rod of solid section, while the latter produces hollow section work piece such as a tube. Aside from the difference in purpose, the plunger in FIG. 2 has a head 2' with a flat, downwardly directed press surface 1'. The block 6' here is presumed to have frustoconical axial faces 14. Another block usable is shown separately in FIG. 3, having a calotte-shaped, lower surface 14'. In either case, whether provided as calotte or as frustoconical protrusion, these axial convexities of the block have base angle  $\sigma$  which is about  $10^\circ$  to  $30^\circ$ . Moreover, the ratio of diameter  $\phi$  to height  $H$  of the cylindrical block is 1:2.5 at the most.

As one can see, in either embodiment, as the plunger is lowered, the compression exerted upon the block 6 commences in the central region along an axis colinear with the direction of motion of the plunger. Basically, that axis is defined as the center of the region of initial compression. There is an initial compression all along the thus defined central core region resulting in a corresponding radial gradient of density. As the pores in this axial region of block 6 are squeezed more, gas if forced to flow into regions in which the pores have been squeezed less. The gas flow follows the resulting radial compression differential, i.e., the gas encapsulated in the pores of block 6 flows from regions of higher density to regions of low density, i.e., from regions of diminished pore volume to regions of less pore volume, which is in radial outward direction.

As the plunger moves down farther, compression continues to propagate radially outwardly from the inner core region of block 6 in outward direction until the material begins to flow for extrusion. The surprising effect is that even if the block has initially a rather high porosity, the gas is pressed out of the block and particularly out of the extruded material to such a degree that a homogeneous, bubble-free work piece can be extruded, either having a hollow section profile as in the equipment shown in FIG. 1 or a solid section profile as in FIG. 2.

A comparison of FIGS. 1, 2 and 3 reveals that the angle relationships as between the several surfaces involved can be established differently with similar results in principle. This includes the possibility of including in the overall consideration, the surface configuration and the material distribution in the block along the contemplated axis of plunger movement. Essential is that inner regions of the block such as an axial core thereof is compressed prior to compression of peripheral regions. The block contour can be directly instrumental in this operation of the extrusion press and in that sense must be regarded as a part thereof. In gen-

eral then, this result can be obtained if the base angles of the several convex projections of plunger and block relative to axial planes are added together (counting flat surfaces as having zero base angle) and if the base angle (or angles) of concave indentations along the axis are subtracted from the sum of the base angles of convex projections. The difference must be positive to obtain the desired radial compression gradient for forcing the encapsulated gas to flow radially outwardly.

The invention is not limited to the embodiments described above but all changes and modifications thereof not constituting departures from the spirit and scope of the invention are intended to be included.

I claim:

1. Apparatus for extruding material, using porous, unclad blocks made of powdery material and having relative density of about 50 to 80 percent, or thereabouts, comprising:

a die member having a cylindrical wall, bottom surface and a central extrusion nozzle in the bottom surface;

a plunger received by the die member for coaction with the die member and defining therewith a receiver cavity for receiving a porous block;

the plunger having a frusto conical or calotte-shaped face as facing the receiver cavity with a particular base angle adjacent the periphery of the plunger relative to an axial plane, the base angle being larger by  $10^\circ$  to  $30^\circ$  than an angle between the bottom surface of the die member adjacent the periphery thereof and an axial plane, the angle between the upper surface of the block in the receiver cavity and the surface of the plunger at the point of contact is larger than the angle between the lower surface of the block and the surface of the die member where in contact therewith, the respective angles taken in any radial plane that includes the axis; so that compressing and degassing of the block upon advancement of the plunger, progresses through the block in radial outward direction and continues in axial extrusion flow through the centrally-axially located extrusion nozzle.

2. Apparatus as in claim 1, the difference between the base angle of the plunger and a corresponding base angle of the die member surface being between  $17^\circ$  and  $22^\circ$ .

3. Apparatus as in claim 1, the cylindrical wall having gas escape channels.

4. Apparatus as in claim 1, the plunger having gas escape channels.

5. Apparatus as in claim 1, there being a mandrel, movably disposed in the plunger, coaxial therewith and with the extrusion nozzle, the mandrel having a conical peak.

6. Apparatus as set forth in claim 5, the apex angle of the cone being  $45^\circ$  to  $70^\circ$ .

7. Apparatus as set forth in claim 5, the apex angle of the cone being about  $60^\circ$ .

8. Apparatus as in claim 1, the internal bottom surface of the die member being conically-shaped with a relatively shallow base angle, the plunger surface being frusto-conical or calotte-shaped with a base angle near the periphery and wall that is larger by at least  $10^\circ$  than said bottom surface angle.

9. Apparatus as in claim 1, the bottom surface angle being between  $0^\circ$  and  $15^\circ$  relative to an axial plane.

10. Apparatus as in claim 9, the bottom surface angle being about  $10^\circ$ .

11. Apparatus as in claim 9, the base angle of the plunger being  $17^\circ$  to  $22^\circ$  larger than the bottom surface angle.